

## UNITED STATES PATENT OFFICE

2,073,831

## COMPOSITION FOR CONDITIONING RUGS

Norman L. Cohen and Columbus W. Vincent, Los Angeles, Calif.

No Drawing. Application September 4, 1935,  
Serial No. 39,190

2 Claims. (Cl. 154—49)

Our invention relates to a composition intended for use as a lining to the back of rugs, carpets and the like, to render them non-slipping on polished floors, to cause them to lie flat on the floor without wrinkling and to impart a greater body and elasticity to them, with the result that the wearing quality of the rugs is improved.

It is known in the art to apply a coating to the back of rugs which renders them non-slipping and while our composition imparts this quality to the rugs, the main object is to increase the durability of the rugs and impart to rugs of medium grade the appearance and "feel" of expensive rugs having a heavy and closely woven nap.

Our invention consists in the composition of matter hereinafter described and pointed out in the claims.

The following is a preferred example of the composition:

|                                                 | Pounds |
|-------------------------------------------------|--------|
| Flour, preferably wheat flour                   | 1      |
| Magnesium chloride solution of 36° Bé. strength | 3      |
| Finely powdered silica                          | 2      |

These ingredients are thoroughly mixed together to form a homogeneous paste which is applied to the back of a rug with a brush or a trowel to form a coating of approximately one-sixteenth inch in thickness. While the coating is still plastic, wood flour or very fine sawdust is applied thereto and the coating is allowed to harden or to set. After the coating has become set the excess of wood flour or sawdust is removed therefrom and a coating of shellac is applied.

In place of the ground silica other fillers, such as clay, sawdust, wood flour, may be used and the proportion may be increased or decreased as desired, or the filler may be omitted altogether. The elasticity of the coating is decreased as the amount of filler is increased. We have found no substitute for magnesium chloride which, as well known, is a hygroscopic substance. Glycerine and calcium chloride have been tested

but we find that the resulting composition is unsatisfactory and that magnesium chloride is essential. It is necessary to apply wood flour or sawdust to the coating while still wet. If the same were omitted and the coating allowed to dry without the application of wood flour or sawdust the coating would in the course of time adhere to the floor. However, in place of applying the wood flour or sawdust to the plastic coating a sheet of burlap may be applied and pressed into it so that it will firmly adhere thereto. The burlap will then prevent the sticking of the rug to the floor and also impart thereto a non-slipping quality.

The proportions of the ingredients stated are those preferred by us although they may be varied, as will be understood by those in the art, and still give good results.

The average thickness of the coating applied to the back of the rug and the like is about one-sixteenth inch but the thickness will vary according to the texture of the rug or carpet. In place of burlap other similar material, such as cheesecloth or coarse absorbent paper, may be used in forming a backing.

As stated above, the silica filler may be omitted. However, I prefer to use the same, especially where in addition to the non-slip qualities of the rug additional weight and body thereof are desired. Furthermore, the use of a heavy filler such as silica will improve the non-wrinkling qualities of the rug.

## We claim:

1. A rug having a lining applied to the back consisting of a composition made of wheat flour, one pound; magnesium chloride 36° Bé., three pounds; and a cellulose material imbedded in the surface of the lining.

2. A rug having a lining applied to the back consisting of a composition made of wheat flour, one pound; magnesium chloride 36° Bé., three pounds; and a sheet of burlap imbedded in the surface of the lining.

NORMAN L. COHEN.  
COLUMBUS W. VINCENT. 45